

1

2,820,766

## LUBRICATING COMPOSITIONS

John Scotchford Elliott and Eric Descamp Edwards, London, England, assignors to C. C. Wakefield & Company Limited, London, England, a British company

No Drawing. Application January 24, 1955  
Serial No. 483,824

Claims priority, application Great Britain  
January 26, 1954

5 Claims. (Cl. 252—46.6)

The present invention comprises improvements in or relating to lubricating compositions and relates particularly to fluid lubricants capable of use over a very wide range of temperatures.

It is an object of the present invention to provide lubricating compositions suitable for use over a wide range of temperatures and under a variety of conditions and suitable for use in internal combustion engines or other mechanisms where high temperatures are involved e. g. in the lubrication of gas turbines, especially the propeller turbine type where the lubricant is required to lubricate not only the bearings but also the reduction gearing, said lubricating compositions also being stable and fluid at low or very low temperatures e. g. down to  $-40^{\circ}$  F. or even  $-80^{\circ}$  F.

It has already been proposed to employ as lubricants (especially suited for use at low temperatures) certain diesters of aliphatic dicarboxylic acids with branched-chain aliphatic alcohols, a number of such esters being described in the Journal entitled "Industrial and Engineering Chemistry," April 1947, p. 484 to p. 497.

These esters possess extremely low pour-points, have excellent viscosity-temperature characteristics and good lubricating properties and have been found very satisfactory lubricants for a variety of instruments such as watches, clocks, aeronautical compasses, gyroscopes, meters, gun-turret mechanisms and a variety of aircraft and other scientific instruments, especially where, as in aircraft, very low temperatures are encountered.

It has also been proposed to stabilise such esters by the addition of antioxidants such as organic amines and phenols of various types.

In our British patent specification No. 696,064 it has been proposed to stabilize these esters by the addition of minor amounts of metal salts of organic dithiophosphoric acids, with or without the further addition of metal salts of oil-soluble petroleum sulphonic acids. By this means the esters could be stabilized against oxidation at relatively high temperatures, and rendered suitable for the lubrication of internal combustion engines and gas turbines.

Recent improvements in the design of gas turbine engines have increased the severity of the demands made upon the lubricant, which must have good oxidation resistance at high temperatures, e. g. of the order of  $200^{\circ}$  C., at the same time being non-corrosive towards metals used in the construction of the turbine engines, e. g. steel, copper, brass, magnesium, aluminium and cadmium-plated steel. It must also possess a high load-carrying capacity, in order to provide adequate lubrication of the reduction gearing in the propeller-turbine type of engines.

In our United States application Serial No. 456,063 we have disclosed the fact that dicarboxylic acid diesters may be very effectively inhibited against oxidation at high temperatures by the addition of minor amounts of hydroxy-substituted diaryl thioethers, and that a still further improvement may be obtained by the inclusion of a basic

2

aliphatic, alicyclic or heterocyclic amine having a boiling point of at least  $140^{\circ}$  C.

It has previously been proposed to increase the load-carrying capacity of dicarboxylic acid diesters by the incorporation therein of trityl phosphate, formerly known as tricresyl phosphate, but in general it has been considered necessary to use a relatively large amount, e. g. of the order of 5%, to produce adequate lubrication of the reduction gearing of propeller type gas turbines.

10 We have now found that by the addition to dicarboxylic acid diesters, of the type described in United States patent application Serial No. 456,063 of both (a) a hydroxy-substituted diaryl thioether, and (b) a neutral organic phosphate or phosphite ester, the load-carrying capacity

15 of these esters can be very substantially enhanced.

The degree of improvement obtained is considerably in excess of that to be expected from consideration of the extreme pressure properties of the two types of additives when used singly. Thus, the hydroxy-substituted diaryl

20 thioethers of the present invention have little or no effect on the load-carrying capacity of the esters while, as has already been stated, fairly large quantities of neutral organic phosphate esters are required to produce adequate lubricating properties under extreme pressure conditions.

25 By the conjoint use of the two types of additives, however, lubricants can be obtained having adequate extreme pressure properties and excellent resistance to oxidation at high temperatures. Furthermore, the total amount of combined additives required to impart a particular degree 30 of load-carrying ability is substantially less than the amount of organic phosphate ester which would be required, if used alone, to give the same result.

According to the present invention there is provided a lubricating composition as claimed in any one of the claims 35 of United States patent application Serial No. 456,063 which lubricating composition has incorporated therein a minor proportion of a neutral organic phosphate or phosphite ester.

The term "neutral ester" used throughout the specification and claims is to be understood as referring to esters having an acidity not exceeding 1 mg. KOH per gm.

The preferred esters have the general formula



where R is an aliphatic or cycloaliphatic hydrocarbon radical having from 2 to 8 carbon atoms, and R<sub>1</sub> and R<sub>2</sub> are the same or different and are branched-chain alkyl or alkyl-substituted cycloalkyl radicals having at least 4 carbon atoms. Examples of the radical R are



55 (CH<sub>2</sub>)<sub>n</sub> (where n is an integer from 2 to 8) and



60 While esters having the above general formula are preferred, it is also within the scope of the invention to employ esters obtained by esterifying the dicarboxylic acids with a mixture of an alcohol and a glycol to give 65 complex esters having the general formula



wherein R, R<sub>1</sub> and R<sub>2</sub> are as defined above and



is a glycol or polyglycol having not more than about 12 carbon atoms.

Other types of complex esters which may be employed are prepared by esterifying a dicarboxylic acid (1 mol) with a glycol (2 mols) and a monocarboxylic acid (2 mols) or with 1 mol each of a glycol, a monocarboxylic acid and a monohydric alcohol.

Esters may be employed derived from succinic, maleic, pyrotartaric, glutaric, adipic, pimelic, suberic, azelaic, sebacic and pinic acids, specific esters being:

Di (1-methyl-4-ethyl octyl) glutarate  
Di (2-ethyl hexyl) adipate  
Di (3-methyl butyl) azelate  
Di (2-ethyl hexyl) azelate  
Di (2-ethyl hexyl) sebacate  
Di (3:5:5-trimethylhexyl) sebacate  
Di (2-ethyl hexyl) maleate  
Di (methyl cyclohexyl) adipate  
2 ethyl hexyl 1-methyl heptyl sebacate  
Di (2-ethyl hexyl) pinate

Whereas the majority of esters falling within the foregoing class possess both a high viscosity index and low pour-point, certain of them e. g. di (1:3 dimethyl butyl) adipate, di (3-methyl butyl) sebacate have relatively high freezing points (above 0° F.), and therefore would not normally be suitable for the purposes of this invention, except in admixture with other esters of lower freezing point.

It will be understood that different esters may be selected according to the conditions under which the lubricant is to be used. Thus for use at very high temperatures it will be preferred to employ the esters of high molecular weight and particularly the higher branched-chain di-esters of azelaic and sebacic acid.

The complex esters which may be employed are preferably prepared by esterifying 2 mols. of the dicarboxylic acid, 2 mols. of the branched-chain aliphatic or alkyl-substituted cycloaliphatic alcohol, and not more than 1 mol. of glycol. Examples of glycols which may be used are ethylene, propylene and hexylene glycols and the polyglycols, e. g. diethylene, triethylene, and tetraethylene glycol.

When a monocarboxylic acid is used in preparing a complex ester this should be a straight or branched-chain aliphatic acid having from 2-10 carbon atoms inclusive.

Specific examples of suitable complex esters which may be employed in accordance with the present invention are:

Ester prepared from ethylene glycol (1 mol), sebacic acid (2 mols) and 2-ethyl hexanol (2 mols).

Ester prepared from triethylene glycol (1 mol) adipic acid (1 mol), n-caproic acid (1 mol) and 2-ethyl hexanol (1 mol).

The hydroxy-substituted diaryl thioethers to be employed in accordance with the present invention have the general formula



wherein the radicals Ar are aromatic nuclei which may be the same or different, but are preferably the same, x, y and z are integers from 1 to 3, and n is zero or an integer from 1 to 6 inclusive. The aryl nuclei may contain as further substituents, alkyl, aryl or ether groups.

The thioethers may be employed in concentrations ranging from 0.05 percent to 5.0 percent, and preferably from 0.1 percent to 2.0 percent, by weight on the weight of the final composition.

Specific examples of hydroxy-substituted diaryl thioethers are:

pp'-Dihydroxy diphenyl thioether

Di(3-methyl-4-hydroxyphenyl) thioether

Di(4-methyl-3-tertiary butyl-2-hydroxyphenyl) thioether

Thioether prepared from tertiary butyl catechol

Di(3-methoxy-4-hydroxyphenyl) thioether  
Thioether prepared from o-phenyl phenol

These compounds can be prepared by well known methods such as by the action of sulphur dichloride on the desired phenol in an inert solvent such as benzene or carbon tetrachloride or, in the case of the last compound, by the action of sulphur dichloride on o-phenyl phenol in the presence of a metal catalyst such as copper powder or iron filings. Their use in mineral lubricating oils has been known for some considerable time, but although possessing antioxidant properties to some degree they have not found wide application in internal combustion engine oils and have been considered inferior to the metal dithiophosphates and other metal-containing additives. It is important that compounds for use in conjunction with the diesters of the present invention should be substantially free from the corresponding di- and polysulphides and from free sulphur.

In view of the fact that these thioethers have had such limited usefulness as antioxidants in mineral oils, it is not a little surprising to find them so effective as antioxidants in diester type lubricants. Moreover, whereas thioethers derived from alkylated phenols, e. g. tertiary butyl phenols and cresols (which themselves have antioxidant properties) have apparently always been preferred for use as antioxidants for mineral oils, we have found that for the purposes of the present invention the best results are obtained by the use of thioethers derived from phenols which are unsubstituted or substituted only by short alkyl radicals such as methyl groups and preferably by not more than one methyl group, although the use of more highly alkylated phenols is not excluded. This preferred class of phenol thioethers have good solubility in the esters of the present invention, but their solubility in most mineral oils is so limited that their use as antioxidants in that connection would hardly be considered.

In addition to the simple thioethers, examples of which have been quoted, it is possible to use polymeric compounds such as those obtained by the action of more than one (but less than 2) mols. of sulphur dichloride, on 2 mols. of a phenol having at least two free ortho- or para-positions in the nucleus.

It will be understood that the compounds selected for use must have adequate solubility in the esters in which they are to be dissolved. Thioethers in which the radicals Ar in the above general formula consist of condensed aryl nuclei, e. g. naphthyl groups, have inadequate solubility unless compensating nuclear alkyl substituents or ether groups are present. Similarly, compounds in which x, y or z are more than 1 tend to lack solubility and must be compensated in the same way. Generally it is preferred to employ compounds in which the radicals Ar are phenyl radicals and x and z are 1 n being zero.

The neutral organic phosphate esters of the present invention have the general formula



where R<sub>1</sub>, R<sub>2</sub> and R<sub>3</sub> are organic radicals and may represent alkyl, aryl, alkaryl or cycloalkyl radicals. Preferably R<sub>1</sub>, R<sub>2</sub> and R<sub>3</sub> will be the same, but if desired mixed esters of phosphoric acid may be employed. It is also within the scope of the invention to employ esters containing more than one phosphate grouping in the molecule, e. g. di-phosphates having the general formula



where R<sub>1</sub> and R<sub>2</sub> are as defined above and R<sub>4</sub> is an alkylene or arylene radical.

Specific examples of neutral organic phosphate esters are:

Trimethyl phosphate  
Triethyl phosphate  
Tri(n-butyl)phosphate  
Tri(2-ethyl hexyl) phosphate  
Triphenyl phosphate  
Tri-o-tolyl phosphate  
Tri-m-tolyl phosphate  
Tri(p-tertiary amyl phenyl) phosphate  
Tri (methyl cyclohexyl) phosphate  
Tri (butoxyethyl) phosphate  
Tetraethyl p-phenylene diphosphate

It will be understood that the particular phosphate esters selected must possess adequate solubility in the dicarboxylic acid diesters in which they are to be used. Consequently, it is preferred in general to employ phosphate esters in which at least one of the radicals  $R_1$ ,  $R_2$  or  $R_3$  contains at least two carbon atoms, or, if the radicals are aryl radicals, that at least one of them, and preferably all three, contains an alkyl substituent.

The neutral organic phosphite esters of the present invention contain at least one atom of trivalent phosphorus attached through oxygen to hydrocarbon radicals, and may have the general formula:



where  $R_1$ ,  $R_2$  and  $R_3$  are organic radicals and may represent alkyl, aryl, alkaryl or cycloalkyl radicals. Preferably  $R_1$ ,  $R_2$  and  $R_3$  will be the same, but if desired mixed esters of phosphorous acid may be employed. It is also within the scope of the invention to employ esters containing more than one phosphite grouping in the molecule.

Since the lubricants are required for use at high temperatures, it is necessary that the phosphate and phosphite esters employed should have boiling points not below about 200° C. and that, when dissolved in the synthetic ester lubricant of the present invention, in the proportions in which they are to be employed, they should not suffer decomposition at this temperature. The neutral organic phosphate esters are thermally stable substances of high boiling-point, even the lowest member of the series, trimethyl phosphate, boiling at 197° C. In employing the phosphite esters, however, it is preferred to select compounds in which the sum of the carbon atoms contained in the radicals  $R_1$ ,  $R_2$  and  $R_3$  is not less than 12.

Any or all of the hydrocarbon radicals of the phosphate or phosphite esters may carry hydrocarbon, ether or ester substituents, provided that these do not impair the stability of the compound at elevated temperatures. The presence of other substituents, however, e. g. halogen and sulphur-bearing groups, other than thioether groups linking two aromatic nuclei, will in general be inadmissible on this account.

One particular class of sulphur-bearing phosphite esters which we have found suitable for the present invention is the phosphite esters of aromatic hydroxy-substituted thioethers, some examples of which, along with other closely related compounds, are described in our United States Patent No. 2,396,839.

Those suitable for use in the present invention have the general formulae:



or



where the radicals  $R$  are hydrocarbon radicals which may carry ether or ester substituents, the radicals  $Ar$  are aromatic radicals which may carry alkyl, ether or ester substituents,  $m$  is zero, 1 or 2, and  $n$  is a small integer from 1 to 3, the sum of  $m$  and  $n$  being 3.

Specific examples of phosphite esters which may be employed in the present invention are:

Tri(n-butyl) phosphite  
Triphenyl phosphite  
5 Tritolyl phosphite  
Tricyclohexyl phosphite  
Di(3 - carbomethoxy - 4 - hydroxyphenyl)thioether ditolyl phosphite.

10 The phosphite esters possess themselves more effective load-carrying properties than the corresponding phosphate esters, and can therefore be used in lesser amounts. The joint use of these phosphite esters with the aromatic hydroxy-substituted thioethers, however, produces a still further improvement in load-carrying ability, and therefore permits a further reduction in the amount of phosphite ester required.

In carrying out the present invention it will be necessary to incorporate the two additives in amounts sufficient to effect a substantial increase in load-carrying 20 capacity over that exhibited by the dicarboxylic acid diesters alone. Thus the thioethers may be employed in concentrations ranging from 0.2 percent to 5.0 percent, and preferably from 0.5 percent to 2.0 percent, by weight on the weight of the final composition, the phosphate esters in amounts of from 0.5 percent to 10 percent but preferably from 1.0 percent to 5.0 percent by weight on the weight of the final composition, and the phosphite esters in amounts of from 0.1 percent to 5 percent but 25 preferably from 0.25 percent to 2.0 percent by weight on the weight of the final composition.

While either the simple diesters of dicarboxylic acids or the complex esters may be employed in accordance with the present invention, these materials have certain 30 limitations. Thus the simple esters have rather too low viscosities to be suitable as such for lubricating the existing types of aircraft gas turbines which normally require a lubricant having a minimum viscosity of 7.5 centistokes at 210° F., whereas the complex esters in 35 general have insufficiently low pour-points which should desirably be of the order of -70° F. or below.

Accordingly, in a preferred form of the present invention the dicarboxylic acid diesters of the type described are thickened to the desired degree by the addition of polymers of esters of acrylic or alkyl-substituted acrylic 40 acids, e. g. methacrylic acid. Compositions of this type 45 can be produced having sufficiently high viscosities combined with very low pour-points.

The polymers are employed in proportions of from 1 percent to 15 percent, preferably from 3 percent to 10 percent, by weight on the weight of the final composition.

Examples of polymers which may be employed are the 50 polymerised n-hexyl, 3:5:5 trimethyl hexyl and lauryl esters of methacrylic acid, and various commercially 55 available materials sold under the trade name "acryloid." It is preferred to use polymers which are not only freely soluble in the diester lubricants but also miscible with mineral oil.

There may also be included in the composition an 60 aliphatic alicyclic or heterocyclic amine having a boiling point of at least 140° C., as disclosed in our United States patent application Serial No. 456,063. Examples of suitable amines which may be used are n-octylamine and higher primary aliphatic amines, dibutylamine, and higher secondary aliphatic amines, cycloaliphatic amines such as dicyclohexylamine, and heterocyclic amines such as the lupetidines and higher homologues of piperidine. Tertiary amines having basic properties may also be employed, e. g. di-n-octylmethylamine and 2:6 lutidine.

65 70 Generally these amines will be employed in relatively small amounts, e. g. from 0.01 to 1.0 percent by weight on the weight of the final composition, and preferably from 0.05 to 0.5 percent by weight on the weight of the final composition.

75 Other additives may be included if desired, e. g. rust

7  
inhibitors such as very small amounts of metal petroleum sulphonates, or other known compounds capable of inhibiting rust formation in presence of water.

It is also within the scope of the invention to include lubricants in which a certain amount of mineral oil is 5 added to the composition.

The amount added and type of mineral oil will depend largely upon the pour-point required for the particular application in mind, but in any case the amount of mineral oil present should not exceed 50% by weight 10 on the weight of the composition.

Where extremely low pour-points of the order of -80° F. are required, the presence of mineral oil may be inadmissible.

Lubricants prepared in accordance with the present invention not only have good extreme pressure properties and resistance to oxidation at high temperatures, but are also relatively non-corrosive to cuprous and other metals, even at very high temperatures, and are free from 15

lacquer and deposit-forming tendencies, and from sensitivity to light.

Specific compositions which may be employed in accordance with the present invention are exemplified in the tables of test results which follow.

To determine the load-carrying capacity of the compositions of this invention, tests were carried out using the well-known Four-Ball Machine, similar to that described by Boerlage in "Engineering," July 13, 1933, volume 136, page 46. This apparatus comprised four steel balls arranged in the form of a pyramid. The top ball was held in a chuck attached to a spindle rotating at approximately 1500 R. P. M. and pressed against the three bottom balls clamped in a stationary ball holder. The balls were immersed in the oil to be tested.

Tests were run for one minute at ambient temperature at a series of different loads.

The ensuing tables illustrate the effectiveness of the compositions of the present invention.

TABLE I

| Test No. | Additives present                      |                              | Initial seizure load, kg. | Mean wear (mms.) at— |         |
|----------|----------------------------------------|------------------------------|---------------------------|----------------------|---------|
|          | Thioether                              | Phosphate or phosphite ester |                           | 100 kg.              | 120 kg. |
| 1.....   | None.....                              | None.....                    | 55-60                     | 2.3                  | W       |
| 2.....   | pp'-Dihydroxydiphenyl thioether (1.0%) | do.....                      | 50-55                     | 2.3                  | 2.6     |
| 3.....   | None.....                              | Tri-m-tolyl-phosphate (3.0%) | 80-85                     | 2.5                  | 2.9     |
| 4.....   | do.....                                | Tri-m-tolyl-phosphate (5.0%) | 75-80                     | 2.6                  | W       |
| 5.....   | pp'-Dihydroxydiphenyl thioether (1.0%) | Tri-m-tolyl-phosphate (3.0%) | 105-110                   | 0.43                 | 2.6     |
| 6.....   | None.....                              | Triphenyl phosphite (1.0%)   | 85-90                     | 2.3                  | 2.8     |
| 7.....   | pp'-Dihydroxydiphenyl thioether (1.0%) | do.....                      | 90-95                     | 2.4                  | 2.5     |
| 8.....   | pp'-Dihydroxydiphenyl thioether (0.5%) | Triphenyl phosphite (0.5%)   | 90-95                     | 2.0                  | 2.4     |

W indicates that welding took place at this load.

The surprising effectiveness of the combined additives (tests 5, 7, 8) as compared with additives used singly (tests 2, 3, 4, 6) can readily be seen from the foregoing results.

TABLE II

[In this series of tests the additives were dissolved in a blend having the following composition: 47% Di(2-ethyl hexyl) sebacate, 47% Di (3:5:5 trimethyl hexyl) sebacate, 6% Polynonyl methacrylate, +0.05% calcium petroleum sulphonate, 0.1% dicyclohexylamine.]

| Test No. | Additives present              |                              | Initial seizure load, kg. | Mean wear (mms.) at— |         |
|----------|--------------------------------|------------------------------|---------------------------|----------------------|---------|
|          | Thioether                      | Phosphate ester              |                           | 100 kg.              | 140 kg. |
| 9.....   | Di(o-cresol) thioether (1.0%)  | None.....                    | Below 50                  | 2.1                  | W       |
| 10.....  | Di(o-cresol) thioether (0.5%)  | Tri-m-tolyl phosphate (3.0%) | 65-70                     | 2.2                  | 2.6     |
| 11.....  | do.....                        | Tri-m-tolyl phosphate (5.0%) | 95-100                    | 2.2                  | 2.6     |
| 12.....  | Di(o-cresol) thioether (0.75%) | Tri-m-tolyl phosphate (2.0%) | 75-80                     | 2.2                  | 2.5     |
| 13.....  | do.....                        | Tri-m-tolyl phosphate (3.0%) | 95-100                    | 2.3                  | 2.55    |
| 14.....  | Di(o-cresol) thioether (1.0%)  | Tri-m-tolyl phosphate (2.0%) | 85-90                     | 2.2                  | 2.6     |
| 15.....  | do.....                        | Tri-m-tolyl phosphate (3.0%) | 95-100                    | 2.2                  | 2.5     |

The di(o-cresol) thioether was a commercially available material consisting mainly of di(3-methyl-4-hydroxy-phenyl) thioether.

The polynonyl methacrylate was 3:5:5 trimethyl hexyl methacrylate polymerised to a degree such that 6% of the polymer when dissolved in a 50/50 blend of the two sebacate esters produced a lubricant having a viscosity of 7.5-8.5 centistokes at 210° F.

The results in Table II illustrate the effect of varying the proportions of two typical additives of the present invention, optimum results being achieved by the use of 0.75% of the thioether with 3.0% of the phosphate ester.

TABLE III

[In this series of tests, the additives were dissolved in a blend having the following composition: 44% Di(2-ethyl hexyl) sebacate, 50% Di(3:5:5 trimethyl hexyl) sebacate, 6% Polynonyl methacrylate.]

| Test No. | Additives present                                       |                                          | Initial seizure load, kg. | Mean wear (mms.) at— |         |
|----------|---------------------------------------------------------|------------------------------------------|---------------------------|----------------------|---------|
|          | Thioether                                               | Phosphate or phosphite ester             |                           | 100 kg.              | 140 kg. |
| 16.....  | Polymeric thioether prepared from p-octyl phenol (1.0%) | None.....                                | 60-65                     | 2.2                  | 2.6     |
| 17.....  | None.....                                               | Tributyl phosphate (2.0%)                | 85-95                     | 2.7                  | 3.5     |
| 18.....  | Polymeric thioether prepared from p-octyl phenol (1.0%) | do.....                                  | 95-100                    | 2.1                  | 2.4     |
| 19.....  | None.....                                               | Tri(2-ethyl hexyl) phosphate (3.0%)      | 70-75                     | 2.45                 | W       |
| 20.....  | pp'-Dihydroxydiphenyl thioether (1.0%)                  | do.....                                  | 90-95                     | 2.2                  | 2.6     |
| 21.....  | None.....                                               | Tri(methyl cyclohexyl) phosphite (0.25%) | 65-70                     | 2.1                  | W       |
| 22.....  | pp'-Dihydroxydiphenyl thioether (1.0%)                  | do.....                                  | 85-90                     | 2.25                 | 2.5     |

The results in Table III further illustrate the advantage of using a combination of the two types of additives. The polymeric thioether employed in tests 16 and 18 was prepared from 1.2 mole of p-octyl (α, γ, γ, γ-tetramethyl butyl) phenol and 1 mol. of sulphur dichloride in benzene solution.

TABLE IV

[This series of tests was designed to provide further examples of typical compositions which may be employed in carrying out the present invention.]

| Test No. | Base blend                                                                       | Additives present                                                                                                                                            | Initial seizure load, kg. | Mean wear, (mm.) at— |         |
|----------|----------------------------------------------------------------------------------|--------------------------------------------------------------------------------------------------------------------------------------------------------------|---------------------------|----------------------|---------|
|          |                                                                                  |                                                                                                                                                              |                           | 100 kg.              | 140 kg. |
| 23.....  | 44% DOS, 50% DNS, 6% PNM                                                         | 1.0% pp'-Dihydroxydiphenyl thioether, 3.0% Tri-m-tolyl phosphate, 0.1% Dicyclohexylamine, 0.05% Calcium petroleum sulphonate.                                | 100-110                   | 0.43                 | 2.6     |
| 24.....  | 44% DOS, 50% DNS, 6% PNM                                                         | 0.5% Di(o-cresol) thioether, 1.0% Di(3-carbomethoxy-4-hydroxyphenyl) thioether ditolyl phosphite 0.1% Dicyclohexylamine, 0.05% Calcium petroleum sulphonate. | 88-90                     | 2.2                  | 2.5     |
| 25.....  | 45% DOA, 45% DNA, 10% Acryloid H. F. 860.                                        | 2% p-Octyl phenyl thioether phosphite, 1% 1:3 Xylen-2-ol thioether.                                                                                          | 125-130                   | 0.47                 | 1.8     |
| 26.....  | 40% Di(2-ethyl hexyl) maleate, 40% Di C <sub>10</sub> adipate, 20% Acryloid 710. | 2% Tributoxyethyl phosphate, 2% Thioether prepared from guaiacol.                                                                                            | 90-95                     | 1.7                  | 2.1     |
| 27.....  | 77% DOA, 17% Oil A, 3.3% Oil B, 2.7% "Polylauryl" methacrylate.                  | 1% Triethyl phosphate, 1.5% Thioether prepared from t-butyl catechol, 0.1% Di-n-octyl methyamine, 0.1% Calcium petroleum sulphonate.                         | 85-90                     | 2.15                 | 2.25    |

In Table IV the abbreviations have the following significance:

DOS=di(2-ethyl hexyl) sebacate  
 DNS=di(3:5:5 trimethyl hexyl) sebacate  
 PNM=polynonyl methacrylate  
 DOA=di(2-ethyl hexyl) adipate  
 DNA=di(3:5:5 trimethyl hexyl) adipate

Di C<sub>10</sub> adipate was a mixture of diesters of adipic acid prepared from mixed branched-chain alcohols having 7-9 carbon atoms.

"Acryloid" HF 860 and 710 were concentrates of polymethacrylate esters in gas oil and mineral oil, respectively, while the "polylauryl" methacrylate was a comparatively low molecular weight co-polymer prepared from the mixed methacrylate esters of commercial lauryl alcohol (83%) and 3:5:5 trimethyl hexanol (17%).

p-Octyl phenol thioether phosphite was prepared by treating 1-mol. of p-octyl ( $\alpha\alpha\gamma\gamma$ -tetramethyl butyl) phenol with 0.5 mol. sulphur dichloride and then treating 3-mols of the resulting thioether with 1-mol. of phosphorus trichloride in presence of 3-mols of pyridine in benzene solution.

Oil A. was a solvent refined mineral oil of viscosity about 150 seconds Redwood at 140° F., and Oil B. a solvent-refined mineral oil of viscosity about 70 seconds Redwood at 140° F.

It is to be understood that the foregoing examples merely afford illustrations of typical compositions of the present invention, and that any of the esters or thioethers exemplified in our United States application Serial No. 456,063 may be employed as alternatives.

The physical properties of certain typical compositions in the preferred viscosity range are quoted in Table V below.

It will readily be seen that these compositions have excellent viscosity-temperature characteristics and very low pour points, in addition to good load-carrying properties.

To determine the oxidation stability of the compositions of this invention at elevated temperatures, a modi-

fication of the well-known British Air Ministry oxidation test was employed. This test was carried out precisely as described in "Standard Methods for Testing Petroleum and its Products," Institute of Petroleum, 1949, Method

40 I. P. 48/44, with the exception that there was present a copper catalyst consisting of a piece of polished copper foil 2 inches x 1 1/4 inches rolled into a cylinder as described in I. P. Method .56/46, this being replaced by a fresh catalyst after every 3 hours. Additionally there were present strips of polished copper foil 6 inches x 1/2 inch suspended in the vapour phase above the oil, the lower portion of the strips being folded into three segments approximately 1 inch long, so that the overall length of the strip above the oil was about 3 inches and the lower end of the strip was 3 1/2 inches above the surface of the oil.

After air blowing, the percentage increase in viscosity and acidity rise were determined together with the percentage of matter insoluble in petroleum ether (boiling point below 40° C.). Also the vapour-phase copper strips were examined for signs of attack by volatile acids, as evidenced by the presence of a green colour.

TABLE V

| Composition of test No. | Viscosity, centistokes at— |         |       |                    | Viscosity index | Pour point    | Open flash point ° F. |
|-------------------------|----------------------------|---------|-------|--------------------|-----------------|---------------|-----------------------|
|                         | 210° F.                    | 100° F. | 0° F. | -40° F.            |                 |               |                       |
| 23.....                 | 7.59                       | 33.4    | 492   | <sup>1</sup> 4,500 | 163             | Below -75° F. | 440                   |
| 24.....                 | 7.95                       | 34.4    | 600   | 6,770              | 164             | do            | 460                   |
| 25.....                 | 7.44                       | 23.07   | —     | —                  | 175             | do            | —                     |

<sup>1</sup> Approximately.

Table VI illustrates the effectiveness of the compositions of the present invention as compared with compositions containing only the phosphate or phosphite esters. The temperature of the tests was 200° C. and the duration 12 hours.

TABLE VI

| Test No. | Ester or ester blend          | Additives                                                                                                                                                      | Percent viscosity change | Acidity (mgs. KOH per gram) | Percent insoluble in petroleum ether (B. B. below 40° C.) | Attack of vapour phase copper strips, observed after— |
|----------|-------------------------------|----------------------------------------------------------------------------------------------------------------------------------------------------------------|--------------------------|-----------------------------|-----------------------------------------------------------|-------------------------------------------------------|
| 28       | 44% DOS, 50% DNS, 6% PNM.     | None                                                                                                                                                           | -10.0                    | 4.5                         | Trace                                                     | 3 hrs.                                                |
| 29       | do                            | 2.0% tri-m-tolyl phosphate, 0.05% calcium petroleum sulphonate.                                                                                                | +7.5                     | 3.5                         | 3.0                                                       | 3 hrs.                                                |
| 30       | do                            | 0.5% triphenyl phosphite, 0.1% dicyclohexylamine.                                                                                                              | +23.8                    | 17.4                        | 0.33                                                      | 6 hrs.                                                |
| 31       | do                            | 0.5% triphenyl phosphite, 0.1% dicyclohexylamine, 1.0% polymeric thioether prepared from p-octyl phenol, 0.05% calcium petroleum sulphonate.                   | +1.6                     | 1.7                         | 0.14                                                      | 6 hrs.                                                |
| 32       | 47% DOS, 47% DNS, 6% PNM.     | 2.0% tri-m-tolyl phosphate, 0.05% calcium petroleum sulphonate, 1.0% pp'-dihydroxydiphenyl thioether.                                                          | +8.0                     | 1.7                         | 0.77                                                      | Absent.                                               |
| 33       | 44% DOS, 48.8% DNS, 7.2% PNM. | 0.5% di-(o-cresol) thioether, 1.0% di(3-carbomethoxy-4-hydroxyphenyl) thioether ditolyl phosphite, 0.05% calcium petroleum sulphonate, 0.1% dicyclohexylamine. | +2.7                     | 2.2                         | —                                                         | Do.                                                   |

It has been found that when an organic phosphite ester is employed in conjunction with a hydroxy-substituted diaryl thioether, particularly good resistance to oxidation is obtained, and such blends are even less prone to stain metals such as copper at high temperatures than the corresponding blends containing phosphate esters or containing only the thioethers. Some further degree of improvement in oxidation and corrosion resistance is obtained by the inclusion of a basic aliphatic, alicyclic or heterocyclic amine having a boiling point of at least 140° C.

It is accordingly particularly preferred to employ compositions containing a hydroxy-substituted diaryl thioether, an organic phosphite ester as hereinbefore defined, and an amine of the type described, such compositions being superior with respect to load-carrying capacity and oxidation and corrosion resistance.

We claim:

1. A lubricating composition comprising a major proportion of at least one ester of the general formula



where R is a radical selected from the group consisting of aliphatic and cycloaliphatic hydrocarbon radicals having from two to eight carbon atoms, and R<sub>1</sub> and R<sub>2</sub> are radicals selected from the group consisting of branched-chain alkyl and alkyl-substituted cycloalkyl radicals having at least four carbon atoms, from 0.2% to 5.0% of a hydroxy-substituted diaryl thioether having the general formula



where R is a member of the group consisting of H and a CH<sub>3</sub> radical and n is an integer not exceeding 4, and from 0.25% to 5.0% of a neutral organic ester selected from the group having the general formulas



and



where R<sub>1</sub>, R<sub>2</sub>, and R<sub>3</sub> are radicals selected from the group consisting of alkyl, aryl, alkaryl and cycloalkyl radicals.

2. A lubricating composition comprising a major proportion of at least one ester of the general formula



where R is a radical selected from the group consisting of aliphatic and cycloaliphatic hydrocarbon radicals having from two to eight carbon atoms, and R<sub>1</sub> and R<sub>2</sub> are radicals selected from the group consisting of branched-chain alkyl and alkyl-substituted cycloalkyl radicals having at least four carbon atoms from 0.2% to 5.0% of a hydroxy-substituted diaryl thioether having the general formula



where R is a member of the group consisting of H and a CH<sub>3</sub> radical and n is an integer not exceeding 4, and from 1.0% to 5.0% of a neutral organic phosphate ester having the general formula



where R<sub>1</sub>, R<sub>2</sub> and R<sub>3</sub> are radicals selected from the group consisting of alkyl, aryl, alkaryl and cycloalkyl radicals.

3. A lubricating composition comprising a major proportion of at least one ester of the general formula



where R is a radical selected from the group consisting of aliphatic and cycloaliphatic hydrocarbon radicals having from two to eight carbon atoms, and R<sub>1</sub> and R<sub>2</sub> are radicals selected from the group consisting of branched-chain alkyl and alkyl-substituted cycloalkyl radicals having at least four carbon atoms from 0.2% to 5.0% of a hydroxy-substituted diaryl thioether having the general formula



where R is a member of the group consisting of H and a CH<sub>3</sub> radical and n is an integer not exceeding 4, and from

## 13

0.25% to 2.0% of a neutral organic phosphite ester having the general formula



where  $\text{R}_1$ ,  $\text{R}_2$  and  $\text{R}_3$  are radicals selected from the group consisting of alkyl, aryl, alkaryl and cycloalkyl radicals.

4. A lubricating composition comprising a major proportion of at least one ester selected from the group consisting of di(2-ethyl hexyl) azelate, di(2-ethyl hexyl) sebacate, di(3:5:5-trimethylhexyl) azelate and di(3:5:5-trimethylhexyl) sebacate, from 0.25 to 2.0% of a neutral organic phosphite ester selected from the group consisting of triphenyl phosphite, trityl phosphite and di(3-carbo-methoxy-4-hydroxy phenyl) thioether ditolyl phosphite, and from 0.2% to 5% of a hydroxy substituted diaryl thioether selected from the group consisting of pp' dihydroxy diphenyl thioether and di(o-cresol) thioether, said thioether being present in sufficient quantity further to increase the load-carrying capacity of the composition.

5. A lubricating composition comprising a major proportion of at least one ester selected from the group consisting of di(2-ethyl hexyl) azelate, di(2-ethyl hexyl) sebacate, di(3:5:5-trimethylhexyl) azelate and di(3:5:5-trimethylhexyl) sebacate; from 1.0% to 5.0% of a neutral

10

15

20

25

## 14

organic phosphate ester selected from the group consisting of tri-m-tolyl phosphate, tributyl phosphate and tri(2-ethyl hexyl) phosphate, and from 0.2% to 5.0% of a hydroxy-substituted diaryl thioether selected from the group consisting of pp' dihydroxy diphenyl thioether and di(o-cresol) thioether, said thioether being present in sufficient quantity further to increase the load-carrying capacity of the composition.

## References Cited in the file of this patent

## UNITED STATES PATENTS

|           |                       |               |
|-----------|-----------------------|---------------|
| 2,139,766 | Mikeska et al. -----  | Dec. 13, 1938 |
| 2,396,839 | Evans -----           | Mar. 19, 1946 |
| 2,499,984 | Beavers et al. -----  | Mar. 7, 1950  |
| 2,639,266 | Dilworth et al. ----- | May 19, 1953  |
| 2,760,934 | Black -----           | Aug. 28, 1956 |

## FOREIGN PATENTS

|         |                     |               |
|---------|---------------------|---------------|
| 455,235 | Great Britain ----- | Oct. 15, 1936 |
|---------|---------------------|---------------|

## OTHER REFERENCES

"Ind. and Eng. Chem.", vol. 39, No. 4 pages 491-497, pages 492 and 493 pertinent.

"Lubrication Engineering," August 1952, pages 177, 178, 179, 197, 198, 199 and 200, page 178 pertinent.